

Patented June 21, 1938

2,121,337

# UNITED STATES PATENT OFFICE

2,121,337

## DYEING MIXED FIBERS

Karl Brodersen and Alfred Peters, Dessau-in-Anhalt, Germany, assignors to General Aniline Works, Inc., New York, N. Y., a corporation of Delaware

No Drawing. Application January 16, 1937, Serial No. 120,904. In Germany January 18, 1936

4. Claims.

(Cl. 8—5)

Our present invention relates to a process for dyeing fabrics or other fibrous materials comprising mixtures of cellulose, preferably regenerated cellulose, such as artificial silk fibers, and animal fibers, preferably wool.

The dyeing of wool in fast tints is known with dyes which are traded under the commercial name Metachrome Dyes (cf. index of Colour Index, 1924 I), that are dyes, generally ortho-hydroxyazo dyes, which are used in presence of metachrome mordant (ammonium sulfate and potassium chromate), thus forming the chromium complex compound of the dye on the fiber.

On the other hand, dyes containing acid groups which in themselves have a certain dyeing capacity on vegetable fibrous material are known to be improved in their fastness to water and washing by treatment before or after the dyeing with compounds having cation activity, for example quaternary bases of various kinds. In the case of Metachrome Dyes the treatment is not applicable for lack of any affinity for vegetable fiber. From their constitution, for example from that of Metachrome Brown (Colour Index, 1923 I No. 101), it could not be supposed that the formation of a sparingly soluble salt decisive for the fixation with a base of high molecular weight would proceed of itself.

The present invention is based on the observation that Metachrome Dyes serve very well for dyeing fibrous materials consisting of cellulose fibrous materials and wool in even shades, if the fibers are pre-treated with a cation-active compound of high molecular weight which in itself has an affinity for artificial cellulosic fibers. It is well known that some groups of dyes having a distinct molecular constitution dye cotton and other cellulosic material without premoderating the fibers, however, until yet no colorless organic compounds were known which are taken up from a dilute aqueous solution and bound by the fibers so that they can be removed neither by washing nor soaping. In the following with the expression "bases having an affinity for artificial fibers" such organic bases of high molecular weight or the salts thereof are meant, which dissolved in water to form solutions of about 0.05 per cent. strength are absorbed by the fibers under corresponding exhaustion of the bath and remain on the fiber even when washing or soaping the latter.

Such bases are, for instance, those which lean in their constitution towards the constitution of direct dyeing dyes, for example, the product of reaction of dichloracetylbenzidine with a trialkyl-

amine or an analogous product of reaction of a tertiary base with the dichloracetyl compound of 4,4'-diaminodiphenylurea.

Particularly advantageous are the bases which contain polyether radicles and guanidine radicles or are derived from guanidine.

These bases are made, for example, by the reaction of the chlorhydrin of a polyglycerol containing, for example, 7 glycerol molecules, with stearylidimethylamine; or by the reaction of di-cyandiamide with a base of high molecular weight, for instance oleylamine, dodecylamine or the like. Derivatives of high molecular weight of guanidine, guanyl urea and the like have similar effect.

We mention, for instance, as especially suitable:—

Oleyl- or stearylbiguanide of the formula



or the corresponding compounds containing another higher alkyl radicle with at least 10 carbon atoms or the biguanides in which the hydrogen of the amino or imino groups is substituted by alkyl or hydroxyalkyl.

Stearylguanidine of the formula



and the corresponding alkyl and hydroxyalkyl derivatives.

The urea derivative of the constitution



With the aid of these bases having an affinity for artificial fibers it becomes possible to uniformly dye mixed fibers consisting of wool and cellulose wool in a single bath process. The fastness to washing, fulling and sweat of the dyes is considerably better than that imparted by other known processes. The application of Monochrome Dyes for the dyeing of such mixed fabrics has become possible owing to this invention.

The mode of operation is preferably as follows:

The mixed fibers are treated for 1 to 2 hours at room temperature in a bath, for example of 1 per cent. strength, of the chloride of the base of high molecular weight; the goods are then

squeezed, rinsed and dyed in the manner usual for dyeing wool with Metachrome Dyes.

The following examples illustrate the invention:—

5. *Example 1.*—A mixed fabric of wool and copper artificial silk is treated for 1 to 2 hours at room temperature in a cold solution of 1 per cent. strength of a quaternary base obtainable by the reaction of the chlorhydrin of a polyglycerol containing about 7 molecules of glycerol with octadecyl-dimethylamine; the goods are then squeezed and rinsed. They are then dyed for an hour and a half at the boil in a bath with 3 per cent. of Metachrome Bordeaux B (Colour Index 1928, No. 107) and 3 per cent. of Metachrome Mordant. There is obtained a dyeing uniform in all fibers. Precipitations do not occur in the liquor.

20. *Example 2.*—A mixed fabric of wool and viscose artificial silk is treated for an hour and a half at room temperature in a liquor which contains 5 grams per liter of oleyl-biguanide, then squeezed and rinsed. It is then dyed at the boil for an hour and a half in a fresh bath with 4 per cent. of Metachrome Brown B (Colour Index 1923 I, No. 101), 4 per cent. of Metachrome Mordant being added. A uniform dyeing of both kinds of fiber is obtained.

25. What we claim is:—

30. 1. The process for dyeing mixed fabrics or other mixed fibrous materials consisting of regenerated cellulose and animal fibers which comprises pre-treating the material with an amidine of the general formula



35. wherein R means an alkyl radicle with at least

10 carbon atoms and x is a connecting radicle of the group consisting of



and then dyeing both the fibers of the mixed material in even shades with an ortho-hydroxyazo dye in the presence of a chromium mordant.

2. The process for dyeing mixed fabrics or other mixed fibrous materials consisting of regenerated cellulose and animal fibers which comprises pre-treating the material with a biguanide of the general formula



wherein R means an alkyl radicle with at least 10 carbon atoms, and then dyeing both the fibers of the mixed material in even shades with an ortho-hydroxyazo dye in the presence of a chromium mordant.

3. The process for dyeing mixed fabrics or other mixed fibrous materials consisting of regenerated cellulose and animal fibers which comprises pre-treating the material with oleyl-biguanide and then dyeing both the fibers of the mixed material in even shades with an ortho-hydroxyazo dye in the presence of a chromium mordant.

4. The process for dyeing mixed fabrics or other mixed fibrous materials consisting of regenerated cellulose and animal fibers which comprises pre-treating the material with oleyl-biguanide and then dyeing both the fibers of the mixed material in even shades in the presence of ammonium sulfate and alkali metal chromate with the dye prepared by coupling diazotized picramic acid with meta-phenylene-diamine.

KARL BRODERSEN.  
ALFRED PETERS.